

1

3,328,211

METHOD OF MANUFACTURING WELDABLE,  
TOUGH AND HIGH STRENGTH STEEL FOR  
STRUCTURE MEMBERS USABLE IN THE AS-  
HOT-STATE AND STEEL SO MADE

Hajime Nakamura, Meguro-ku, Tokyo-to, Japan, assignor to Ishikawajima-Harima Jukogyo Kabushiki Kaisha, Tokyo-to, Japan, a company of Japan  
No Drawing. Filed Nov. 18, 1964, Ser. No. 412,231  
Claims priority, application Japan, Dec. 5, 1963,  
38/65,481  
4 Claims. (Cl. 148—12)

This invention relates to a weldable, tough and high strength steel for structure members usable in the as-hot-worked state and method of manufacture therefor.

There are a number of steels available today on commercial market that purport to have a tensile strength of 60 kg./mm.<sup>2</sup> class together with ductility, toughness and weldability that are adequate for fabrication of large steel structures such as ships, buildings, pressure vessels or bridges. Here, a term "60 kg./mm.<sup>2</sup> class" is used to designate a range for tensile strength which is defined as between 58 kg./mm.<sup>2</sup> and 70 kg./mm.<sup>2</sup>, both limits inclusive, in accordance with Japanese standards.

However, I am, as yet, unaware of one that is capable of developing the desired set of mechanical properties, namely high strengths, both yield and tensile, coupled with good ductility and/or toughness without sacrificing one in favor of the other, if left in the as-worked, for example, as-rolled state. Therefore, heat treatment of one variety or another has generally to be applied to those steel stocks, despite considerable increase in price, to make the strength, ductility, toughness and weldability all adequate for a structure member steel.

Thus, an object of this invention resides in the provision of inexpensive, weldable, tough and high strength steel for structure members that is perfectly usable in its as-hot-worked state, namely without any subsequent or independent heat treatment, having a set of mechanical properties which is characterized by strength, ductility and toughness all maintained at a high level. Another object is to determine the proper composition for the steel described above so that the steel may possess the set of mechanical properties as desired in the as-hot-worked state when manufactured properly. The third is to give the proper method of hot-working for the particular steel described above, by which combination, namely proper hot-working on steel of proper composition, it is only possible to obtain the set of mechanical properties desired. Other objects of this invention will in part be mentioned in due course, and yet others will either be self-explanatory or be readily understood or appreciated by those who are skilled in the art.

More specifically, this invention relates to a weldable, tough and high strength steel for structure member that is capable of developing a tensile strength of at least 58 kg./mm.<sup>2</sup> but not over 70 kg./mm.<sup>2</sup>, yield ratio, the ratio of yield strength to tensile strength, of at least 72%, a ductility of at least 25% in elongation on gauge length of four times the specimen diameter at room temperature, and a notch impact toughness of at least 80 ft.-lb. or 13.8 kg.-m./cm.<sup>2</sup> at 0° C. by 2 mm. V notch Charpy test piece.

It also relates to a steel composition in the final product analysis which comprises by weight percent: carbon 0.08-0.30%, silicon 0.02-0.60%, manganese 0.5-2.50% nitrogen less than 0.045%, the whole or at least 0.010% of which is to be bound to aluminum in the form of precipitated aluminum nitride of 0.03-0.12%, the rest to any one or combination selected from the group com-

2

posed of: columbium less than 0.20%, titanium less than 0.12% and zirconium less than 0.20%; free uncombined nitrogen less than 0.004%, free metallic aluminum dissolved in matrix as solid solution (solid solution metallic aluminum) less than 0.15%, as well as at least one complementing alloying element selected from the group consisting of: nickel 0.10-1.0%, chromium 0.10-1.0% molybdenum 0.05-1.0%, copper 0.05-1.0%, vanadium 0.005-0.30%, boron 0.0005-0.01%; the balance substantially all iron with incidental or unavoidable impurities.

This invention relates further to a method of manufacture for weldable, tough and high strength steel or structure member characterized by the set of mechanical properties defined earlier in the as-hot-worked state, the method comprising hot-working the steel in any manner in the temperature range of 1200°-700° C., starting at a temperature not above 1200° C. and finishing at not below 700° C., giving the steel a reduction in thickness, calculated on the final thickness of the product, of at least 20% in the temperature range below 1000° C. in one or more passes, thereafter cooling the steel.

As mentioned earlier briefly, in order to obtain a set of mechanical properties which is as good as or even better in the as-hot-worked state than that may be realized after heat treatment, not only the hot-working procedure but also the composition of the steel stock must be carefully controlled. Namely, this invention is based on the discovery of the conditions governing both those ends. In the steel composition: Carbon, the foremost alloying element for steel, is necessary by at least 0.08% to ensure the 60 kg./mm.<sup>2</sup> class tensile strength when co-prescribed with other ingredients, but tends to spoil the weldability of the steel when present in excess of 0.30%, the preferred range falling in from about 0.10% to 0.25%.

Silicon is added as deoxidizing agent for which at least 0.02% is needed, but tends to excessively harden the matrix by solid solution effect and to affect unfavorably the ductility when present by more than 0.60%, the preferable range being from about 0.3 to 0.5%.

Manganese, which is also an active deoxidizer, is an element that is capable of hardening the steel without impairing the weldability, for which purpose at least 0.5% is needed. However, when present in excess of 2.5%, it tends to stabilize the lower bainite in the as-hot-worked steel to give rise to a higher strength at a considerable expense in the ductility and toughness. Thereupon, the manganese content is limited to from 0.5 to 2.5%, of which 0.5 to 2.0% is the preferred range.

Aluminum nitride component of at least 0.03% on nitrogen of about 0.01% is necessary to ensure a high ductility and toughness. However, we have observed in attempting to provide precipitated aluminum nitride more than about 0.12%, or, in terms of nitrogen bound to aluminum, 0.041%, the nonmetallic inclusions, particularly oxides of aluminum and silicon that are inevitably retained in the steel, increases rapidly and the cleanliness, and with it the ductility and toughness, of the steel correspondingly declined. The favorable effect the precipitated aluminum nitride exerts on the toughness and ductility itself, on the other hand, tends to saturate as the content approaches this 0.12% level.

Some solid solution metallic aluminum content is unavoidable insofar as more aluminum must be provided over what is needed for the stoichiometric combination with available nitrogen to ensure the desired aluminum nitride content, but it is an unwelcome constituent for the steel because aluminum dissolved in solid solution with



TABLE 1A

| No. | AlN   | Met. Al | Nitride Former Other than Al   | Al in AlN | Tot. N | F. N  | N in AlN | N in Other Nitride |
|-----|-------|---------|--------------------------------|-----------|--------|-------|----------|--------------------|
| 1   | 0.052 | 0.051   |                                | 0.035     | 0.021  | 0.004 | 0.017    |                    |
| 2   | 0.032 | 0.033   |                                | 0.021     | 0.014  | 0.003 | 0.011    |                    |
| 3   | 0.055 | 0.003   | Cb, 0.019                      | 0.037     | 0.021  | 0.001 | 0.018    | 0.002              |
| 4   | 0.052 | 0.016   | Zr, 0.038                      | 0.035     | 0.024  | 0.002 | 0.017    | 0.005              |
| 5   | 0.036 | 0.028   | Zr, 0.047; B, 0.001            | 0.024     | 0.017  | 0.001 | 0.012    | 0.004              |
| 6   | 0.049 | 0.034   | Zr, 0.023                      | 0.033     | 0.021  | 0.003 | 0.016    | 0.002              |
| 7   | 0.055 | 0.019   | V, 0.04; Ti, 0.006             | 0.037     | 0.022  | 0.002 | 0.018    | 0.002              |
| 8   | 0.052 | 0.012   | V, 0.04; Cb, 0.046             | 0.035     | 0.024  | 0.002 | 0.017    | 0.005              |
| 9   | 0.047 | 0.013   | Cb, 0.041; Zr, 0.093; B, 0.001 | 0.032     | 0.023  | 0.000 | 0.015    | 0.008              |
| 10  | 0.003 | 0.031   |                                | 0.002     | 0.008  | 0.007 | 0.001    |                    |
| 11  | 0.005 | 0.009   |                                | 0.003     | 0.007  | 0.005 | 0.002    |                    |

TABLE 2.—HOT ROLLING DATA

| Steel | Soaking Temperature, °C. | Rolling Schedule          |                            |                             |
|-------|--------------------------|---------------------------|----------------------------|-----------------------------|
|       |                          | Starting Temperature, °C. | Finishing Temperature, °C. | Finishing Reduction Percent |
| 1     | 1,150                    | 1,100                     | 850                        | 40                          |
| 2     | 1,170                    | 1,120                     | 830                        | 35                          |
| 3     | 1,150                    | 1,090                     | 820                        | 58                          |
| 4     | 1,180                    | 1,100                     | 840                        | 50                          |
| 5     | 1,150                    | 1,110                     | 840                        | 45                          |
| 6     | 1,150                    | 1,090                     | 800                        | 25                          |
| 7     | 1,150                    | 1,090                     | 820                        | 34                          |
| 8     | 1,140                    | 1,100                     | 810                        | 49                          |
| 9     | 1,100                    | 1,070                     | 790                        | 44                          |
| 10    | 1,140                    | 1,100                     | 800                        | 41                          |
| 11    | 1,320                    | 1,270                     | 950                        | 10                          |

<sup>1</sup> Reduction in thickness calculated on product, obtained at temperatures below 1,000° C.

TABLE 3.—MECHANICAL PROPERTIES OF  $\frac{1}{2}$ " THICK PLATE

| Steel | Yield Strength, kg./mm. <sup>2</sup> | Tensile Strength, kg./mm. <sup>2</sup> | Elongation, Percent | $\frac{V}{E}$ , <sup>2</sup> kg.-m/cm. <sup>2</sup> | Yield Ratio, Percent |
|-------|--------------------------------------|----------------------------------------|---------------------|-----------------------------------------------------|----------------------|
| 1     | 52.4                                 | 65.6                                   | 25.4                | 16.6                                                | 79.9                 |
| 2     | 48.8                                 | 67.6                                   | 25.0                | 14.2                                                | 72.2                 |
| 3     | 53.4                                 | 64.7                                   | 29.0                | 19.3                                                | 82.7                 |
| 4     | 49.2                                 | 68.5                                   | 27.2                | 14.6                                                | 72.3                 |
| 5     | 48.5                                 | 62.2                                   | 26.8                | 16.1                                                | 77.9                 |
| 6     | 49.6                                 | 65.1                                   | 27.4                | 15.6                                                | 76.2                 |
| 7     | 49.8                                 | 65.2                                   | 32.8                | 17.8                                                | 76.6                 |
| 8     | 60.0                                 | 68.7                                   | 32.0                | 19.4                                                | 82.7                 |
| 9     | 46.8                                 | 60.7                                   | 32.0                | 18.2                                                | 77.3                 |
| 10    | 36.0                                 | 58.4                                   | 32.8                | 13.3                                                | 61.7                 |
| 11    | 42.1                                 | 65.3                                   | 25.3                | 7.5                                                 | 64.4                 |

<sup>1</sup> Gauge length 40 mm., 10 mm. diameter specimen.

<sup>2</sup> Charpy 2 mm. V notch specimen, at 0° C.

It will be seen in those tables that the steels with chemical composition according to this invention and prepared in accordance with the method of the invention all exhibit the set of mechanical properties specified. It is further noted that Steel 10, which was prepared according to the method of the invention from commercial Cr-Mo type steel stock, compares very favorably with Steel 11, which is in fact a high quality low-manganese grade commercial steel. However, the low temperature notch toughness of Steel 10 fails to attain the 80 ft.-lb. (13.8 kg.-m/cm.<sup>2</sup>) level, or the yield ratio the 72% requirement, because the aluminum nitride content is not as much as required in this invention. Those results shown by Steels 1 to 9 of this invention are simply compared with those of Steels 10 and 11 for the superiority to be appreciated.

It will further be seen that a wide variety of combinations of mechanical properties fit for particular service requirements can be gained by properly selecting the chemical composition and/or manufacturing procedures. For example, Steels 1, 3 and 8 may advantageously be used for structures designed on the yield stress basis for their high yield points; here the presence of columbium, partly in the form of columbium nitride existing along with aluminum nitride, is appreciated, while the application of Steels 3, 7, 8 and 9 may be quite profitable in the low temperature service structures for their high notch toughness.

15 Although only the flat-rolling process was used in describing the method of the invention, we hold no special preference for it in the hot-working method. Forging, swaging, section-rolling or any other known processes of hot-working are equally satisfactory inasmuch as the working is carried out in accordance with the method of this invention.

Having described heretofore the principles and applications of this invention, I do not wish to be confined to the factual examples shown, but only by the claims as set forth.

I claim:

1. A method of manufacturing weldable, tough and high strength steel for structure members usable in the as-hot-worked state, said steel consisting of carbon 0.08-0.30%, silicon 0.02-0.60%, manganese 0.5-2.5%, nitrogen less than 0.045%, at least 0.010% of which is to be bound to aluminum in the form of precipitated aluminum nitride of 0.03-0.12%, the rest to any one selected from the group composed of: columbium less than 0.20%, titanium less than 0.12% and zirconium less than 0.20%, and a combination thereof; free uncombined nitrogen less than 0.004%, free metallic aluminum dissolved in the matrix as solid solution less than 0.15%, as well as at least one complementing alloying element selected from

35 the group consisting of: nickel 0.10-1.0%, chromium 0.10-1.0%, molybdenum 0.05-1.0%, copper 0.05-1.0%, vanadium 0.005-0.30%, boron 0.0005-0.01%; the balance substantially all iron with incidental and unavoidable impurities, the method consisting of heating the steel to a soaking temperature in the range of 1100°-1200° C., hot-working the steel in the temperature range of 1200°-700° C., starting the hot working at a temperature not above 1200° C. and finishing at a temperature not below 700° C., giving the steel a reduction in thickness, calculated on the final thickness of the product, of at least 20% in at least one pass in the temperature range below 1000° C., and thereafter cooling the steel.

2. The method according to claim 1, wherein the steel consists of carbon 0.10-0.25%, silicon 0.3-0.5%, manganese 0.5-2.0%, precipitated aluminum nitride 0.03-0.12%, metallic aluminum dissolved in the matrix as solid solution less than 0.15%, at least one from: the group consisting of columbium less than 0.20%, titanium less than 0.12%, zirconium less than 0.20%, free uncombined nitrogen less than 0.004%, as well as at least one from: the group consisting of nickel 0.2-0.8%, chromium 0.3-0.8%, molybdenum 0.1-0.6%, copper 0.1-0.8%, vanadium 0.02-0.1%, boron 0.0005-0.005%; the balance substantially all iron with incidental and unavoidable impurities.

3. A weldable, tough and high strength steel for structure members usable in the as-hot-worked state having a tensile strength of at least 58 kg./mm.<sup>2</sup> but not over 7 kg./mm.<sup>2</sup>, a yield ratio of at least 72% as measured on gauge length of four times the specimen diameter, and a notch impact toughness of at least 80 ft.-lb. or 13.8 kg.-m./cm.<sup>2</sup> at 0° C. as measured by 2 mm. V notch Charpy test piece, said steel consisting of the ingredients and having been made by the steps defined in claim 1.

4. A weldable, tough and high strength steel for structure members usable in the as-hot-worked state having a tensile strength of at least 58 kg./mm.<sup>2</sup> but not over 70 kg./mm.<sup>2</sup>, a yield ratio of at least 72%, a ductility at room temperature of at least 25% as measured on guage length of four times the specimen diameter, and a notch impact toughness of at least 80 ft.-lb. or 13.8 kg.-m./cm.<sup>2</sup> at 0° C. as measured by 2 mm. V notch Charpy test piece, said steel consisting of the ingredients and having been made by the steps defined in claim 2. 10 15

|           |         |               |       |          |
|-----------|---------|---------------|-------|----------|
| 3,155,496 | 11/1964 | Nakamura      | ----- | 75-124   |
| 3,155,549 | 11/1964 | Nakamura      | ----- | 75-124 X |
| 3,173,782 | 3/1965  | Melloy et al. | ----- | 75-123   |
| 3,259,488 | 7/1966  | Nakamura      | ----- | 75-124   |

## FOREIGN PATENTS

|         |         |                |
|---------|---------|----------------|
| 786,993 | 11/1957 | Great Britain. |
| 808,556 | 2/1959  | Great Britain. |
| 830,669 | 3/1960  | Great Britain. |
| 904,886 | 9/1962  | Great Britain. |

## References Cited

## UNITED STATES PATENTS

|           |         |                    |       |           |
|-----------|---------|--------------------|-------|-----------|
| 3,010,822 | 11/1961 | Altenburger et al. | ----- | 75-123    |
| 3,155,495 | 11/1964 | Nakamura           | ----- | 75-124 15 |

DAVID L. RECK, Primary Examiner.

H. F. SAITO, Assistant Examiner.